

# UNITED STATES PATENT OFFICE.

CECIL VILHELM SCHOU, OF COPENHAGEN, DENMARK.

## SMOKE-GENERATOR FOR SHRAPNEL, SHELLS, &c.

SPECIFICATION forming part of Letters Patent No. 728,737, dated March 24, 1903.

Application filed September 12, 1902. Serial No. 123,1205. (No model.)

*To all whom it may concern:*

Be it known that I, CECIL VILHELM SCHOU, a subject of the King of Denmark, and a resident of Copenhagen, Denmark, have invented certain new and useful Improvements in Smoke-Generators for Shrapnel, Shells, and the Like, of which the following is a specification.

This invention relates to shrapnel and projectiles which explode after they leave the gun and usually at the instant they hit the target, the object of the invention being to provide a practicable material which will evolve a dense smoke of distinctive color or character when the shell explodes and which can readily be seen at the gun from which the shell is discharged to enable the gun-crew to determine distances. Such material should, preferably, not add or detract from the explosive or penetrative force of the shell, but simply develop into smoke under the action of the intense heat of the ordinary explosive mixture used in the shell. It has been proposed to use material for this purpose heretofore; but so far as known by me the materials heretofore proposed have been expensive or have other objectionable features, which have prevented them from being largely used. The need of such a smoke-generator is due to the fact that the ordinary explosive mixtures do not yield sufficient smoke or a smoke of such color as to be discerned at the greater distances.

The material which I have invented for the purpose named consists of sublimated zinc and flower of sulfur or pulverized brimstone, the proportions being such as to present about

as many atoms of metallic zinc as sulfurous atoms. These two materials will give, by chemical combination, a sulfid of zinc, which is totally transformed by the intense heat produced by the explosive mixture of the shell into a white cloud of smoke which can be seen from a great distance. Owing to the presence of oxidized zinc and sometimes other foreign substances in the powder of zinc, it becomes necessary to determine the actual amount of metallic zinc, so that the proportions named may be accurately obtained. By weight the proportions are, substantially, of sublimated zinc sixty-five and flowers of sulfur thirty-two. An advantage of this mixture is that it does not become deteriorated and is not an element of danger when being prepared or, later, when in the shells, the point at which it will burn being very high.

Having thus described my invention, I claim—

1. A smoke generator or producer for shrapnel, shells and similar projectiles, consisting of a mixture of sublimated zinc and flowers of sulfur, substantially as described.

2. A smoke-generator for shrapnel, shells and similar projectiles, consisting of sublimated zinc and flowers of sulfur in the proportions, by weight, substantially of sixty-five and thirty-two respectively.

In testimony that I claim the foregoing as my invention I have signed my name in presence of two subscribing witnesses.

CECIL VILHELM SCHOU.

Witnesses:

VIGGO BLOM,  
F. A. USPUY.